

## UNITED STATES PATENT OFFICE

2,321,280

## SAFETY FUEL

Cecil L. Brown, Baton Rouge, La., assignor to  
 Standard Oil Development Company, a corpora-  
 tion of Delaware

No Drawing. Application December 7, 1938,  
 Serial No. 244,357

10 Claims. (Cl. 44—80)

The present invention is directed to fuels for aircraft, known as safety fuels.

Safety fuels are characterized by a high flash point, a high octane number, good volatility and gum stability. For example, a good safety fuel should have a Tag closed cup flash point of 100° F. or more, an octane number of about 100, and a boiling range of about 300—400° F. It should have also the other characteristics of good aviation gasoline, such as a good gum stability and a good breakdown test.

The desirability of using a safety fuel has long been apparent in the aviation industry. Thus far, however, the industry has not universally adopted any standard safety fuel, primarily because there has been no available source of supply of such fuels at a suitable price.

It has hitherto been proposed to produce safety fuels by several methods such as the destructive hydrogenation of selected distillates or crudes, the extraction with sulfur dioxide of certain distillates or crudes, and the catalytic cracking under selected conditions of such extracts. The fuels produced by the first method are rather high priced due to the limited quantity of suitable raw materials. The fuels produced by the latter two methods have so low an initial octane number and so low a lead susceptibility that the amount of lead required to convert them into 100 octane fuels makes their cost well-nigh prohibitive.

I have now found that fuels having satisfactory characteristics for safety fuels such as high initial octane number, high lead susceptibility and suitable boiling range can be produced from C<sub>4</sub> iso-hydrocarbons. For example, the copolymerization of normal and isobutylene yields a heavy hydrocarbon fraction which, when hydrogenated, boils between about 300 and 385° F., has a high flash point and a high octane number.

I have found that by cutting the mixture of hydrocarbons produced by the reaction between an isoparaffin and an olefin, such as isobutane and normal or isobutylene, at about 300° F., it is possible to produce a heavy fraction having a boiling range of from about 300 to 400° F. which has a Tag closed cup flash in excess of 100° F., a high initial octane number, and a high lead susceptibility. A particularly desirable safety fuel, according to the present invention, is a blend of the last mentioned heavy fraction of alkylation product with hydrogenated tri-isobutylenes boiling between about 330 and 380° F., with the latter constituting from 10 to 50% of the blend. These types of fuels are disclosed and claimed in

copending application Serial No. 457,947, filed July 22, 1942.

The basic materials for the safety fuels of the present invention are available in large quantities and the methods by which they are converted into the desired safety fuels are not costly. For example, practically all refinery gases resulting from cracking processes of various types contain substantial percentages of isobutylene and normal butylenes which can be caused to co-polymerize by being contacted with sulfuric acid of a strength ranging from 60 to 75% at a temperature between about 175 and 250° F. This process is usually conducted with a view of producing dimer, and to this end it is customary to recycle trimer to the reaction chamber. As the result of the present invention, this process can be carried out with a view of producing the highest yield per pass of high boiling hydrocarbons, whereby the efficiency of the method is increased. If desired, the process can be so controlled as to produce mainly trimer by allowing the concentration of dimer to build up in the reaction chamber.

There are large reservoirs of isobutane which can be utilized as sources of raw material for the second embodiment of the present invention. The reaction between isobutane and the olefins of refinery gases proceeds with ease at normal room temperatures in the presence of concentrated sulfuric acid. This reaction, which yields a product containing C<sub>5</sub>—C<sub>8</sub> hydrocarbons, can be made to yield a product boiling mainly within the safety fuel range by recycling C<sub>5</sub>—C<sub>8</sub> hydrocarbons to the reaction zone.

The fuels of the present invention do not per se have an octane number of 100. The co-polymer of isobutylene and normal butylenes, when hydrogenated, has an octane number of about 90 which can be brought to 99.5 with 3 cc. of tetraethyl lead per gallon. Likewise, the high boiling alkylation fraction, especially when blended with about 40% of hydrogenated triisobutylene, has a clear octane number of about 90 which can be raised to 100 with 3 cc. of tetraethyl lead per gallon.

The safety fuel of the present invention is preferably composed entirely of the reaction product of an iso-C<sub>4</sub> hydrocarbon with a different C<sub>4</sub> hydrocarbon. It may be mentioned, however, that, when the fuel is an alkylation product, it may be produced from isopentane or isohexane as well as from isobutane. Likewise, olefins other than the butylenes may be employed. In any case, the fuel, as previously men-

tioned, may contain substantial quantities of hydrogenated triisobutylene. Other suitable blending agents are alkylated aromatics boiling between 300 and 400° F. Typical examples of such alkylated aromatics are ethyl benzene, propyl benzene, isopropyl benzene, methyl ethyl benzene, o, m, p, trimethyl benzene, 1, 2, 3, trimethyl benzene 1, 2, 4, trimethyl benzene 1, 3, 5, secondary butyl benzene, isobutyl benzene, tertiary butyl benzene, and methyl isopropyl benzene, p.

Alternatively, a fraction boiling between 300 and 400° F. of the product resulting from the alkylation of aromatics with olefins may be employed.

The characteristics of typical examples of aviation safety fuel according to the present invention are given in the following table. Fuel A of this table was prepared by reacting isobutylene and normal butylene in the presence of sulfuric acid of a strength of about 70% at a temperature of 170° F., recovering from the product a fraction boiling above 300° F. and hydrogenating this fraction by contacting it with a catalyst composed of  $MoO_3$ ,  $ZnO$  and  $MgO$  at a temperature of 500-600° F. and under a pressure of 3000 pounds per square inch in the presence of a large excess of hydrogen.

Fuel B was prepared by reacting isobutane and the iso- and normal butylene in  $C_4$  refinery cut in the presence of sulfuric acid having a strength of 98% at a temperature of 70° F. and under a pressure sufficient to maintain the reactants in the liquid state and recovering from the product a fraction having the boiling range shown in the table.

Fuel C was prepared by blending with fuel B hydrogenated triisobutylene boiling between 330 and 358° F., the latter constituting 40% of the blend.

|                          | Fuel A   | Fuel B   | Fuel C   |
|--------------------------|----------|----------|----------|
| A. P. I. gravity.....    | 52.7     | 55.8     | 55.8     |
| Color Saybolt.....       | +19      | +26      | +27      |
| Aniline point.....°F.    |          | 182      | 189      |
| Sulfur.....percent.      | 0.01     | 0.02     | 0.008    |
| Doctor.....              | Passes   | Passes   | Passes   |
| Corrosion.....cu. dish   | Passes   | Passes   | Passes   |
| Gum.....cu. dish, mgs.   |          | 3.6      | 3.8      |
| Acid heat.....°F.        | 2        | 1        | 2        |
| Bromine.....No.          | 3        | 1        | 2        |
| Flash.....Tag closed cup | 112      | 103      | 104      |
| Reid vapor pressure..... | Below 1# | Below 1# | Below 1# |
| Army octane number.....  | 89.4     | 77.0     | 85.3     |
| Dto. -3.0 cc. TEL.....   | 99.5     | 96.4     | 100      |
| Initial.....°F.          | 304      | 323      | 328      |
| 5 percent.....           | 319      | 336      | 336      |
| 10 percent.....          | 324      | 341      | 340      |
| 30 percent.....          | 336      | 351      | 347      |
| 50 percent.....          | 345      | 357      | 352      |
| 70 percent.....          | 352      | 363      | 355      |
| 90 percent.....          | 362      | 373      | 361      |
| Final.....°F.            | 384      | 393      | 385      |
| Recovery.....percent.    | 98.0     | 98.0     | 98.0     |
| Residue.....do.....      | 1.0      | 1.0      | 1.0      |

The nature and objects of the present invention having thus been described, what is claimed as new and useful and is desired to be secured by Letters Patent is:

1. A safety fuel boiling substantially completely between about 300° and 400° F., having a flash point of at least 100° F. by the closed cup method, composed predominantly of the paraffinic compounds formed by the reaction between isobutane and a  $C_4$  olefin and containing sufficient antiknock agent to bring its octane number to about 100.

2. A safety fuel boiling substantially completely between about 300° and 400° F., having a flash point of at least 100° F. by the closed cup method, composed predominantly of the paraffinic compounds formed by the reaction between isobutane and isobutylene, and containing sufficient antiknock agent to bring its octane number to about 100.

3. A safety fuel boiling substantially completely between about 300° and 400° F., having a flash point of at least 100° F. by the closed cup method, composed of a mixture of alkylated aromatics and paraffinic compounds formed by the reaction between isobutane and a  $C_4$  olefin and containing sufficient antiknock agent to bring its octane number to about 100.

4. A safety fuel boiling substantially completely between about 300 and about 400° F. having a flash point of at least 100° F. by the closed cup method composed predominantly of saturated branched chain hydrocarbons of the above stated boiling range which are separated from the products produced by reacting isopentane and at least one mono-olefin under alkylating conditions in the presence of an alkylation catalyst.

5. A safety fuel according to claim 4 in which sufficient anti-knock agent is added to raise the octane number to about 100.

6. A safety fuel boiling substantially completely between about 300 and about 400° F. having a flash point of at least 100° F. by the closed cup method composed predominantly of saturated branched chain hydrocarbons of the herein stated boiling range and which are separated from the product produced by reacting isopentane and at least one  $C_4$  olefin under alkylating conditions in the presence of an alkylation catalyst.

7. A safety fuel boiling substantially completely between about 300 and about 400° F. having a flash point of at least 100° F. by the closed cup method composed predominantly of saturated branched chain hydrocarbons of the herein specified boiling range and which are separated from the product produced by reacting isopentane and isobutylene under alkylating conditions in the presence of an alkylation catalyst.

8. A safety fuel according to claim 7 in which sufficient anti-knock agent is added to raise the octane number to about 100.

9. A safety fuel boiling substantially completely between about 300° F. and about 400° F., having a flash point of at least 100° F. by the closed cup method, composed predominantly of paraffinic reaction products of an isoparaffin taken from the group consisting of isobutane and isopentane and an olefin and containing sufficient antiknock agent to bring the octane number to about 100.

10. A safety fuel boiling substantially completely between about 300° F. and about 400° F., having a flash point of at least 100° F. by the closed cup method, composed predominantly of paraffinic reaction products of an isoparaffin taken from the group consisting of isobutane and isopentane and at least one butene and containing sufficient antiknock agent to bring the octane number to about 100.